

Nov. 7, 1939.

G. WILMANNS ET AL

2,179,238

MANUFACTURE OF POLYCHROME PICTURES

Filed April 4, 1936



Gustav Wilmanns  
Wilhelm Schneider  
Ernst Bauer

Inventors

<sup>their</sup>  
by Attorneys  
Shutte and Joslin

Patented Nov. 7, 1939

2,179,238

# UNITED STATES PATENT OFFICE

2,179,238

## MANUFACTURE OF POLYCHROME PICTURES

Gustav Wilmanns, Wolfen, Kreis Bitterfeld, and Wilhelm Schneider and Ernst Bauer, Dessau, Germany, assignors, by mesne assignments, to Agfa Ansco Corporation, Binghamton, N. Y., a corporation of Delaware

Application April 4, 1936, Serial No. 72,718  
In Germany April 10, 1935

10 Claims.

(Cl. 95—6)

Our present invention relates to the manufacture of polychrome pictures and more particularly to the manufacture of polychrome pictures from photographic silver halide emulsions.

5 One of its objects is to provide a process for the production of improved polychrome pictures from silver halide emulsions. Another object are the improved photographic silver halide emulsion layers containing a component which 10 produces color in the developer. Further objects will be seen from the detailed specification following hereafter.

It is known that layers of silver halide emulsion can be developed in color by permitting the 15 products of reaction, produced during the development from developer constituents which have a free amino-group, to condense with reactive phenols or amines to form quinone-imine dyestuffs as for instance indoamines, indoanilines, and indophenols. Dyestuff formation also occurs with bodies which contain a reactive methylene group in which case azomethines are produced. Since, however, in the methods hitherto applied for development in color the component which produces color is incorporated in the developer the method leads merely to monochrome pictures. Attempts to incorporate in the emulsion layer the substance that produces the color have failed, particularly when several 20 layers are used one above the other for producing a polychrome picture. In this case either in applying the second or a later layer to the first layer, or in bringing the material arranged in one or more layers into the developing solution, 25 the components in the emulsion that produce color and are generally soluble in alkali, pass into the adjacent layer into the developer.

The present invention relates to a process in which such diffusion is prevented and the components are fixed in the several colloidal layers. 40 For this purpose there is introduced into the dyestuff component a group which lends the component substantive character with respect to the binding agent of the silver halide emulsion, that is to say, which prevents diffusion in the binding agent of the silver halide emulsion. By introduction of such a group the component can be dissolved in a water-soluble or alkali-soluble form in the colloid without fear that in 45 the finished photographic material the component will diffuse into the adjacent layer or layers. The substantive character produced by introduction of the group can be further strengthened by means of an agent which has a precipitating action on or by means of a group which increases the molecular dimensions of the component. Agents which have a precipitating action are, for instance, diphenylguanidine and diphenylbiguanidine. Groups which increase the 55 molecular dimensions of the component are, for

instance, amino groups, benzoyl groups and benzoyl amino groups which are introduced between the component which produces color and the component which imparts substantive character.

5 Suitable groups for imparting such substantive character and therefore suitable for introduction into the hitherto known color-producers are, for example, diphenyl, dianisidine, toluidine, diphenylcarboxylic acid, diamino-benzoylamino-di-phenyl, stilbene, di-aminostilbene, diamino-benzoylaminostilbene, azoxybenzene, hydroxynaphthoic acid-amides, such as 2,3-hydroxynaphthoic acid and 4-(2,3)-hydroxynaphthoylamino-aniline, diaryl-ureas such as diamino-diphenyl-urea, diamino-benzoylamino-diphenyl-urea, and the urea from amino-benzoylamino-o-sulfanilic acid, benzthiazole, dehydrothiotolidine, amino-naphthols, such as 2-amino-5-naphthole-7-sulfonic acid and 2-aminobenzoylamino-5-naphthole-7-sulfonic acid, terephthaloylbisacetic ester, 10 2,3-hydroxyanthracene-carboxylic acid, 2,3-hydroxycarbazole-carboxylic acid, aminochrysene, aminopyrene, and aminonaphthylene-oxide, or the like. Components for producing color into 15 which these groups are to be introduced are, for example, phenols such as m-aminophenol, o-o'-dinaphthole, o-hydroxydiphenyl, thymol, 2,5-di(phenylamino)-phenol, aniline, naphthols, such as  $\alpha$ -naphthol,  $\alpha$ -hydroxynaphthoic acid, chloronaphthole and trichloronaphthole, naphthylamine, for instance,  $\alpha$ -naphthylamine, amino-naphthols, for instance, 1,5-aminonaphthole, and all compounds which contain a reactive methylene group, for instance aceto-acetic esters, 20 for instance, bromo-acetoacetic acid ester and acetoacetic anilide, cyano-acetic esters, for instance, cyanacetic acid ester, benzoyl-acetic esters, for instance, benzoylacetic anide, hydroindenes, for instance, diketohydrinden, pyrazolones, such as phenylmethylpyrazolone and 1-phenyl-3-phenylpyrazolone, coumaranones, malonic acid anilide,  $\omega$ -cyanaceto-phenon, hydroxythionaphthene, and the like.

The following example illustrates the invention:

The three-color layers, which may be arranged on one or both sides of the support, contain as components for producing color:

1. Para-(oxynaphthoylamino)-1-phenyl-3-methyl-5-pyrazolone for red development,
2. Terephthaloylbisacetic acid-anilide for yellow,
3. 3,5-di(phenylamino)-phenol for blue-green.

The alkali salts of these bodies, dissolved in 55 methanol, are stirred into a gelatin solution of 10 per cent strength in the proportion of 1 gram to 50 cc. of the gelatin solution, and the solution is then mixed with 100 cc. of silver halide emulsion. A suitable developer is one consisting of 60

1 gram of diethylamino-anilide-hydrochloride, 6 grams of potassium carbonate and 100 cc. of water, to which sulfite may be added, if desired.

As it is shown in the example aforesaid, the substantive groups may be introduced into the color components by means of an amide linkage. Thus, for instance, hydroxynaphthoic acid chloride may be condensed with 1-p-amino-phenyl-3-methyl-5-pyrazolone so that an amide is formed by the carboxyl group of the hydroxynaphthoic acid and the amino group of the pyrazolone. The substantive groups may be introduced also by means of an ester linkage. It is again possible to directly connect the compounds.

The single figure of the accompanying drawing shows a film in accordance with the invention having a support 1 coated with a silver halide emulsion layer 2 containing a color component having a group which imparts substantive to the binding agent.

What we claim is:

1. A light-sensitive material for color photography comprising a silver halide emulsion containing a dyestuff component for color forming development having attached thereto a group which lends said component substantive character with respect to the binding agent of the silver halide emulsion and further containing a compound having a precipitating action on said dyestuff component.

2. In a process of producing photographic color pictures the step which comprises treating an exposed photographic material having a silver halide emulsion containing a component for dyestuff forming development having attached thereto a group which lends said component substantive character with respect to the binding agent of the silver halide with a solution of a developing substance having an unsubstituted amino-group in order to produce the color.

3. In a process of producing photographic colored pictures, the step which comprises developing by means of an amino-developer an exposed photographic material having a silver halide emulsion containing a dyestuff component for color forming development having attached thereto a group which renders said component fast to diffusion in the binding agent of the silver halide emulsion, said group comprising at least two organic rings.

4. In a process of producing photographic colored pictures, the step which comprises developing by means of an amino-developer an exposed photographic material having a silver halide emulsion containing a dyestuff component for color forming development having attached thereto a group which renders said component fast to diffusion in the binding agent of the silver halide emulsion, said group comprising at least ten carbon atoms.

5. A light-sensitive material for color photography comprising a silver halide emulsion containing a mononuclear phenolic dyestuff component for color forming development having attached thereto a group which lends said component substantive character with respect to the binding agent of the silver halide emulsion, said group comprising at least two 6-membered aromatic rings.

6. The process as defined in claim 3, wherein at least 2 of said rings are selected from the class consisting of fused rings and rings joined together by a linkage selected from the class consisting of a nuclear carbon to nuclear carbon linkage, an acid amide linkage, a  $-\text{CH}=\text{CH}-$  linkage, a  $-\text{NON}-$  linkage, and a  $-\text{NHCONH}-$  linkage.

7. The process as defined in claim 3, wherein at least 1 of said rings is a heterocyclic ring.

8. A light-sensitive material for color photography comprising a silver halide emulsion containing a dyestuff component for color forming development, selected from the class consisting of mononuclear phenolic dyestuff components and acyl acetic ester dyestuff components, having attached thereto a group which renders said component fast to diffusion in the binding agent of the silver halide emulsion, said group comprising at least two 6-membered aromatic rings.

9. A light-sensitive material as defined in claim 8, wherein the component for color forming is an aceto acetic ester.

10. A light-sensitive material as defined in claim 8, wherein the component for color development is a cyanacetic ester.

GUSTAV WILMANNS.  
WILHELM SCHNEIDER.  
ERNST BAUER.

50